

Oct. 13, 1959

M. E. NORDBERG

2,908,838

APERTURE MASK TREATMENT TO PREVENT CATHODE POISONING

Filed Feb. 25, 1957

Fig. 1



Fig. 2



INVENTOR,  
MARTIN E. NORDBERG  
BY  
Clarence R. Petty, Jr.  
ATTORNEY

# United States Patent Office

2,908,838

Patented Oct. 13, 1959

1

2,908,838

## APERTURE MASK TREATMENT TO PREVENT CATHODE POISONING

Martin E. Nordberg, Corning, N.Y., assignor to Corning Glass Works, Corning, N.Y., a corporation of New York

Application February 25, 1957, Serial No. 642,073

5 Claims. (Cl. 313—85)

This invention relates to an improved perforate mask for assembly in a cathode ray tube of the type used in multicolor television receivers and to a cathode ray tube embodying such mask.

Certain types of multicolor television systems operate on the general principle of emitting a stream of electrons from one or more electron guns mounted in the neck of a cathode ray tube and directing such stream of electrons through a perforate mask onto a viewing screen composed essentially of a phosphor pattern deposited on a face plate or panel forming the opposite end of the tube. The perforate mask, for example the present tube component commonly referred to as a shadow or aperture mask, is positioned transversely of the electron path intermediate the electron gun and screen to intercept all electrons striking the mask and thereby form a plurality of electron beams passing through the apertures or perforations in the mask to the pattern of phosphors on the face of the tube. Multicolor television systems of this sort are described in detail in the patent literature such as United States Patent No. 2,625,734 to Harold F. Law.

The apertures in such a mask are small and closely spaced and must be formed with an extreme degree of accuracy to produce a clear, well-defined picture. Thus specifications of a typical mask call for apertures 10 mils in diameter and uniformly spaced 28 mils center to center, and a mask thickness of 55 mils with the aperture dimensions being held to a tolerance of  $\pm 0.5$  mils. The inherent difficulties in producing and handling such a mask are quite readily apparent. Furthermore it is frequently necessary to sag or otherwise form such a mask to a definite curvature.

Etched metal masks have been proposed, but their use requires a great deal of care to avoid warpage, bending, or other physical damage during production and subsequent handling. It has been recognized that a mask composed of ceramic material such as glass should be highly desirable, but, until discovery of the chemical method of machining glass described in United States Patent No. 2,628,160 issued to S. D. Stookey, no satisfactory method existed for producing such masks. It was naturally assumed that, if a mask of glass or other ceramic could be satisfactorily produced, its use in a tube should present no particular problem since glass is used in construction of the tube envelope itself and other ceramics are widely used in electronic tubes.

Once glass masks were successfully made by the Stookey method, it was quite unexpectedly found that tubes embodying such masks in their assembly tended to fail shortly after being placed on life test. Extensive investigations into these tube failures indicated that the failure was due to a foreign material poisoning the cathode of the electron gun during its operation and that this foreign material was in some manner coming from the glass mask. It is then a primary purpose of the present invention to provide chemically perforated, glass masks free from such prior deficiencies and capable of

2

being used in cathode ray tubes for absorption of electrons.

By way of illustration the present invention is described with reference to the accompanying drawings in which,

Fig. 1 is a schematic representation, largely in section, of a cathode ray tube and,

Fig. 2 is an enlarged fragmentary view in section of a perforate mask in accordance with the invention.

10 The cathode ray tube, schematically represented in Fig. 1 and designated by the numeral 10, has an electron gun 12 mounted in the tube neck 14 and a viewing screen 16 composed of a phosphor coating 18, of suitable composition and pattern for multicolor television, applied to the inside surface of transparent face plate or panel 20 which forms the opposite, enlarged end of the tube. The phosphor coating is applied in any known manner in a dot, stripe or other type of pattern suitable for the purpose. Perforate glass mask 22 is mounted intermediate electron gun 12 and screen 16, by any suitable conventional means, not specifically shown.

20 In Fig. 2 a fragment of mask 22 is shown greatly exaggerated to better illustrate chemically perforated apertures 26 which are too small and too numerous to be satisfactorily shown in a full view such as Fig. 1. In accordance with the exemplary mask specifications referred to earlier, the diameter of apertures 26 is 10 mils and they are spaced 28 mils apart center to center. For 30 purposes of illustration mask 22 is shown flat, and apertures 26, as shown, are formed normal to the electron intercepting surface. As a practical matter mask 22 will frequently have imparted to it a definite curvature and apertures 26 may be formed at angles up to 25° or so from normal depending on the location and geometry of the tube components. The angle of each aperture will be such as to provide alignment of electron gun, apertures and screen elements for proper screen scanning.

35 In accordance with my present invention an electron absorbing, perforate mask, for assembly and use in a cathode ray tube, is produced by firing a chemically perforated glass mask in a reducing atmosphere containing free hydrogen. The effectiveness of this treatment indicates that the poisoning agent released during electron bombardment of an untreated glass mask is oxygen, and that preliminary firing of the glass in the presence of hydrogen, that is in accordance with the present invention, causes such oxygen to combine with the hydrogen or to otherwise be rendered unavailable for subsequent release. This theory is supported by tests in which 40 gases evolved from various glasses under electron bombardment have been collected and analyzed, such test glasses including both hydrogen-fired and untreated glass capable of being chemically perforated.

45 The atmosphere in which the glass is fired preferably contains at least 25% hydrogen. While smaller amounts may be effective the amount of time required is usually too long for practical purposes. The effectiveness of the hydrogen firing increases with temperature and it is therefore desirable to employ the maximum firing temperature possible without distortion of the glass. This maximum temperature will depend in large measure on the viscosity characteristics of the glass and will generally be on the order of 100° C. below the glass softening point. However higher temperatures may be employed where, 50 in the course of the heat treatment, the glass is converted into a glaceramic material, that is a material consisting of an inorganic, crystalline skeleton or network with or without a glassy matrix. It is preferable therefore to use glasses of this nature which are described in 55 explicit detail in U.S. patent application S.N. 538,510 filed October 10, 1955, in the name of Stanley D. Stookey

and assigned to the assignee of the present application.

By way of specifically illustrating the present invention and its effectiveness, reference is made to a test conducted on glass test pieces approximately  $\frac{3}{4}$  of an inch square by 50 mils thick and prepared from a glass composed essentially of 79.5% SiO<sub>2</sub>, 10% Li<sub>2</sub>O, 5% K<sub>2</sub>O, 4% Al<sub>2</sub>O<sub>3</sub>, and 1% ZnO and containing minor amounts of Ag, Au and CeO<sub>2</sub> as photosensitizing agents and Sb<sub>2</sub>O<sub>3</sub> as a firing agent. These glass test pieces were given the standard thermal treatment which precedes etching of this glass in accordance with the Stookey method, that is the samples were held 40 minutes at 580° C. and thereafter 30 minutes at 650° C. Following this preliminary heat treatment, certain of the glass test pieces were given an identical heat treatment in an atmosphere containing 30% hydrogen and 70% nitrogen, while the remainder were held free of further firing for comparison purposes. One of each type was then placed in a special electron bombardment apparatus, designed to permit collection and analysis of gas evolved as well as a record of cathode operation, and was subjected to electron bombardment under cathode ray tube operating conditions of 25 kilovolts. In the course of this test it was observed that, when a test piece which had not been fired in hydrogen was being bombarded, there was a steady evolution of gas, including a substantial proportion of oxygen, and a corresponding steady diminishing of cathode effectiveness. In contrast to this, no appreciable evolution of oxygen was observed during bombardment of a test piece previously fired in hydrogen, and operation of the cathode remained normal during such bombardment, thus illustrating the effectiveness of hydrogen treatment on this glass.

The commercial significance of these results was confirmed in a subsequent actual tube test. In this test a cathode ray tube, having mounted therein a chemically perforated glass mask fired in a hydrogen containing atmosphere, was still successfully operating at the conclusion of an arbitrary thousand-hour test period, whereas similar tubes containing identical glass masks, except for the hydrogen treatment, fail at intervals from a hundred to five hundred hours with an average life around three hundred hours.

While the invention has been described essentially with

relation to what is currently known as a shadow mask, it will be appreciated that it is not restricted to a mask having the specific size and pattern of perforations in such mask, but is equally applicable to other types of perforate masks as well regardless of perforation pattern or size.

What is claimed is:

1. A mask adapted to absorb electrons in a cathode ray tube and having a plurality of perforations extending therethrough which transmit electrons to form a corresponding plurality of electron beams, said mask consisting of a thin sheet of perforated glass having a surface incapable of evolving cathode poisoning gas upon being subjected to electron bombardment.
2. In a cathode ray tube assembly including an image reproducing screen, an electron emission means, and a perforate mask interposed between the emission means and screen to form a plurality of electron beams by selective electron absorption, a perforated glass mask having a surface incapable of evolving cathode gas upon being subjected to electron bombardment.
3. A method of treating a perforate glass mask for incorporation into a cathode ray tube which includes firing such mask in a reducing atmosphere composed in part at least of hydrogen and forming a surface on said glass which is capable of absorbing electrons without appreciable evolution of cathode poisoning gas.
4. The method of claim 3 wherein the reducing atmosphere contains at least 25% hydrogen.
5. In the production of a glass mask adapted to absorb electrons in a cathode ray tube, the method which comprises treating the mask in a hydrogen-containing atmosphere at an elevated temperature and forming thereon a surface capable of absorbing electrons without appreciable evolution of cathode poisoning gas.

#### References Cited in the file of this patent

#### UNITED STATES PATENTS

|           |           |       |               |
|-----------|-----------|-------|---------------|
| 2,279,168 | Kalischer | ----- | Apr. 7, 1942  |
| 2,347,982 | Bachman   | ----- | May 2, 1944   |
| 2,392,099 | Pollard   | ----- | Jan. 1, 1946  |
| 2,777,084 | Lafferty  | ----- | Jan. 8, 1957  |
| 2,805,360 | McNaney   | ----- | Sept. 3, 1957 |